

# UNITED STATES PATENT OFFICE.

PIERRE-ARMAND BRANGIER, OF AGNEW, AND JOHN J. FAULKNER, OF BERKELEY,  
CALIFORNIA.

## REDUCTION OF ZINC OXIDS.

No. 906,191.

Specification of Letters Patent.

Patented Dec. 8, 1908.

Application filed May 29, 1907, Serial No. 376,426. Renewed July 28, 1908. Serial No. 445,745.

*To all whom it may concern:*

Be it known that we, PIERRE-ARMAND BRANGIER, a citizen of France, residing at Agnew, Santa Clara county, and JOHN J. FAULKNER, a citizen of Great Britain, of Berkeley, Alameda county, and State of California, have invented new and useful Improvements in the Reduction of Zinc Oxids, of which the following is a specification.

10 Our invention is designed to provide an economic and rapid process of producing metallic zinc; and it consists substantially in passing hydrogen or carbureted hydrogen gases over a heated mass of zinc oxid.

15 It also comprises details of construction which will be more fully explained in the following specification.

In carrying out our process, we first heat zinc oxid in an iron retort to a temperature sufficient to volatilize the zinc oxid. After this temperature is attained, we pass hydrogen or carbureted hydrogen over the heated ore.

The carbureted hydrogen gas may be produced either from coal gas, or from crude petroleum; and passing over the zinc, which is at substantially its volatilizing temperature, the zinc oxid will be wholly reduced, and the metallic zinc, and carbon monoxid 30 or carbon dioxid are formed. The character of this last product depends entirely on the composition of the hydrocarbon used in the process, and whether such hydrocarbon be manufactured from coal, crude petroleum, 35 or if it is a natural gas, the reason for this being the different combinations in which hydrocarbons appear.

The hydrocarbon or hydrogen being passed over the heated zinc oxid as above described, 40 the union of the gas and the volatilized zinc oxid reduces the zinc to a metallic state, and it is collected in a receiver or condenser in

a molten condition, as metallic zinc said receiver having a temperature sufficient to retain the zinc in a molten state. This temperature at the condenser is necessary to be maintained, otherwise much material in the form of small grains of crystalline zinc or zinc powder may be formed.

The following reactions are believed to take place during the process:



Having thus described our invention, what we claim and desire to secure by Letters Patent is—

1. The process herein described for producing metallic zinc, said process consisting in heating the oxid of zinc to a volatilizing temperature, then mixing therewith a body of hydrocarbon gas or vapor, transferring the volatilized zinc to a chamber where the 60 temperature is reduced to the point of fluidity of the zinc.

2. The process herein described for producing metallic zinc from an oxid thereof, 65 said process consisting in heating the oxid to a temperature which will volatilize the metal, and introducing therewith a gas or vapor containing hydrogen, and finally reducing the temperature to recover the metallic zinc in a fluid form.

In testimony whereof we have hereunto set our hands in presence of two subscribing witnesses.

PIERRE-ARMAND BRANGIER.  
JOHN J. FAULKNER.

Witnesses:

S. H. NOURSE,  
FREDERICK E. MAYNARD.